

Oct. 20, 1925.

1,557,730

F. S. SMITH  
METHOD OF PRODUCING A FIBROUS MASS IMPREGNATED WITH A  
PHENOLIC CONDENSATION PRODUCT  
Filed Feb. 15, 1921

*Fig. 1.*



*Fig. 2.*



INVENTOR.

Franklin S. Smith  
BY  
Cyrus N. Anderson

ATTORNEY.

Patented Oct. 20, 1925.

1,557,730

# UNITED STATES PATENT OFFICE.

FRANKLIN S. SMITH, OF PHILADELPHIA, PENNSYLVANIA, ASSIGNOR TO THE PRODUCTS PROTECTION CORPORATION, OF NEW YORK, N. Y., A CORPORATION OF DELAWARE.

## METHOD OF PRODUCING A FIBROUS MASS IMPREGNATED WITH A PHENOLIC CONDENSATION PRODUCT.

Application filed February 15, 1921. Serial No. 445,114.

To all whom it may concern:

Be it known that I, FRANKLIN S. SMITH, a citizen of the United States, and a resident of Philadelphia, in the county of Philadelphia and State of Pennsylvania, have invented an Improvement in the Method of Producing a Fibrous Mass Impregnated with a Phenolic Condensation Product, of which the following is a specification.

My invention relates to the method of producing material consisting of organic fibers such as jute, cotton, etc., impregnated with a phenolic condensation product, for instance, bakelite; the said product being either in the intermediate or B form, in which it is moldable, or in the final or C form.

One of the objects of my invention is to provide a novel method whereby an improved material consisting of organic uncut or natural fibers impregnated with an intermediate phenolic condensation product, as bakelite B, the said fibers so impregnated being moldable may be produced.

A still further object of the invention is to provide an improved and novel method whereby a material may be produced which in its final condition, in which the condensation product has been converted into the solid C form, possesses among other characteristics those of high tensile and dielectric strength (the latter being uniform in all directions), toughness and requisite homogeneity.

Another object of the invention is to provide a practical and workable method for the production of material of the character above mentioned.

Still another object of the invention is to provide a method whereby flexible uncut fibers, preferably organic, may be impregnated with a phenolic condensation product and molded into such form as may be desired.

No attempt will be made at this point to point out all of the objects and advantages of my invention, but other objects and advantages thereof will be pointed out in the detailed description thereof which follows or will be apparent from such description.

In the carrying out of my invention I take the spun fibers of jute (which I have

found to be especially well adapted to the purposes of my invention), cotton or other like or equivalent materials, and impregnate them with an initial condensation product, such as bakelite A. One way of effecting this is to take the fibers in the form of yarn (by which term I include string, thread, cord, twine, etc.) which has been wound into balls, and place the latter in a suitable receptacle containing an initial phenolic condensation product, as bakelite A, in solution in a mixture of ethyl or methyl alcohol and benzol in proportions which may range from thirty to seventy per cent. of alcohol by volume and from seventy to thirty per cent. of benzol to effect impregnation thereof. In practice the fiber balls of yarn are placed in a strong receptacle which is then hermetically sealed and the solution of bakelite A supplied to such receptacle under a pressure of approximately ten thousand pounds per square inch. The yarn is found to be fully or sufficiently impregnated within a period of a few minutes, five to ten, although the fiber balls of yarn may be allowed to remain in the solution for a longer period if desired. Such longer or additional treatment does not appear to have any beneficial effect; neither does it appear to have any deleterious or injurious effect. If the pressure is decreased the time required to effect complete impregnation is increased and by leaving the balls of fiber in the solution for a sufficient length of time, say a few days, impregnation may be effected at atmospheric pressure. The balls of yarn are then removed from the solution and the solvent removed therefrom. To effect rapid and efficient removal of the solvent not only from the surface but from the interior of the impregnated yarn or string it is then unwound from the said ball onto a reel, drum or the like, or a ball, and as it passes from the first named ball to the latter or to a reel or drum it is subjected to electric current of a voltage such as will produce a voltage gradient at the surface of the yarn or string sufficient to form corona thereon. The gradient necessary to form corona is 31.5 Kv./Cm. at standard temperature and barometric pressure. The first named ball from which the yarn is unwound is insu-

100  
105

lated and the yarn which is unwound therefrom is passed or moved in contact with an insulated metal terminal of suitable form having connection with one end of the secondary of a transformer the other end of which is grounded. Specifically, as illustrated in the drawing in which Fig. 1 is a view partly in section and partly in side elevation of a portion of apparatus which 10 may be employed in the carrying out of the invention and Fig. 2 a transverse sectional view taken on the line 2—2 of Fig. 1, a plurality of metal rings 1 (of large diameter as compared with the yarn or string) 15 are secured upon a metal bar 2 which is insulated and which is connected to one end of the secondary 2 of a transformer, the primary of which is shown at 4. The opposite side or end of the secondary is 20 grounded, as indicated at 6, and is connected to a rod or wire 7 which extends through the said rings and is concentric therewith. The said rod or wire 7 is supported by any suitable support of insulating material, not shown. The yarn 8 is drawn through these rings in contact with any point thereof and corona is produced thereon as indicated by the divergent lines at 9. The charging of the yarn and the 25 producing or forming of corona thereon causes the yarn or string to vibrate very rapidly and effects removal of the solvent therefrom. The yarn, before reaching the rings (or other form of contacts) is conducting, but after leaving the same is non-conducting, it having been freed of the solvents. The rings or other suitable contacts are spaced short distances from each other, and by varying the number thereof 30 40 the speed at which the yarn can be unwound from the first named reel may be varied. By increasing the number so that the yarn is kept in contact with the contact members for a longer period as it travels 45 along, the speed of movement thereof may be increased. While it is possible to convert the phenolic condensation product from the A to the B form by the action of the electric current such practice is not followed because of the time which would be 50 required. In order, therefore, to convert the said product from the A to the B form the impregnated yarn, after the last mentioned step of the treatment, is heated to a temperature of from 75° to 80° centigrade, 55 which effects conversion to the intermediate or B stage. A much higher temperature may be employed but its use requires much greater skill and experience.

50 The yarn or string thus treated and when cold is hard and wiry, but upon being heated to about eighty degrees centigrade and above becomes soft and pliable and may be molded into any shape desired.

65 In employing the material consisting of

yarn of organic spun fiber impregnated with bakelite B for the manufacture of articles of whatever kind may be desired, and for which the said material may be suitable, an amount of the said yarn sufficient for the purpose in hand is packed into molds, previously heated. The mold is of a temperature above eighty degrees centigrade, preferably around one hundred and thirty degrees. The material when packed into the molds thus heated very quickly becomes soft and pliable, whereupon the plunger or die of a press into which the mold has previously been placed is moved down into the mold and the said material is subjected to pressure to form it into the shape of the mold which may be of the shape required for the purpose in hand. The pressure employed may range from one thousand to five thousand pounds per square inch. The pressure and the temperature are maintained for a period of time, depending upon the thickness of the article being molded or formed, during which the bakelite B is converted into bakelite C.

The impregnated yarn is packed indiscriminately that is, in a tangled or haphazard condition, into the mold so that one portion of yarn may be and is interlocked with another portion, the fibers thereof being thus interlocked and bound together.

The term "bakelite" employed in the specification and claims is used in a descriptive and not in a limiting sense and is intended to comprehend phenolic condensation products suitable for the purpose herein described and which possess or have the characteristics above indicated.

Having thus described my invention, what I claim and desire to secure by Letters Patent, is:

1. The method of producing a string of organic material impregnated with an intermediate phenolic condensation product which comprises, first, impregnating the same with an initial phenolic condensation product in solution and thereafter charging the same with an electric current of high tension and producing corona thereon.

2. The method of producing a string of organic material impregnated with bakelite B, which comprises first impregnating the same with bakelite A in solution, thereafter charging the same with an electric current of high tension and producing corona thereon, and simultaneously moving the string forward past and in contact with the charging means.

3. The method of producing a string of organic material impregnated with bakelite B, which comprises the dissolving of bakelite A in a suitable solvent, thereafter impregnating the said string with the solution thus formed, subjecting the same to the ac-

tion of a high tension electric current for removing the solvent from the said string and thereafter converting the bakelite from the A to the B form.

5 4. The method of producing a string of organic material impregnated with an intermediate phenolic condensation product, which comprises the dissolving of an initial phenolic condensation product in a suitable 10 solvent, thereafter producing corona discharge upon the said string to remove the solvent therefrom and converting the initial to an intermediate phenolic condensation product.

15 5. The method of producing a solid fibrous mass of the character described, which comprises impregnating organic fiber with a solution of bakelite A, thereafter subjecting the said fiber to an electric charge of high 20 tension and producing corona thereon to remove the solvent, thereafter applying heat to convert the bakelite A into bakelite B, and thereafter placing the said impregnated fiber in a mold and simultaneously subjecting it to pressure and heat at a temperature 25 above eighty degrees centigrade.

6. The method of producing a solid fibrous mass of the character described comprising the impregnating of a string of organic fibers with bakelite A in solution,

thereafter charging the said string with an electric current of high tension and producing corona thereon and simultaneously removing the solvent therefrom and also simultaneously moving the string forward, 35 converting the bakelite A into bakelite B and thereafter packing the said string into a mold and subsequently simultaneously subjecting it to pressure and heat at a temperature above eighty degrees centigrade, 40 substantially as described.

7. The method of producing a fibrous solid mass of the character described, comprising dissolving bakelite A in a mixture of alcohol and benzol, placing organic fiber string 45 within the solution thus formed under pressure, thereafter removing the said string from the said solution and charging the same with an electric current of high tension to effect removal of the solvent, converting the bakelite A into bakelite B, the said string being thereafter packed into a mold and subsequently simultaneously subjected to the action of pressure and heat at a temperature above eighty degrees centigrade. 50

In testimony that I claim the foregoing as my invention, I have hereunto subscribed my name this 7th day of February, A. D. 1921.

FRANKLIN S. SMITH.